



US006061077A

# United States Patent [19]

Kashiwaya et al.

[11] Patent Number: 6,061,077

[45] Date of Patent: May 9, 2000

## [54] THERMAL HEAD

[75] Inventors: **Makoto Kashiwaya; Junji Nakata**,  
both of Kanagawa, Japan[73] Assignee: **Fuji Photo Film Co., Ltd.**, Kanagawa,  
Japan

[21] Appl. No.: 09/366,728

[22] Filed: Aug. 4, 1999

## [30] Foreign Application Priority Data

Aug. 4, 1998 [JP] Japan ..... P10-220358

[51] Int. Cl.<sup>7</sup> ..... B41J 2/335

[52] U.S. Cl. ..... 347/203

[58] Field of Search ..... 347/203

## [56] References Cited

## FOREIGN PATENT DOCUMENTS

61-53955 11/1986 Japan ..... B41J 3/20

4-62866 10/1992 Japan ..... B41J 2/335  
7-132628 5/1995 Japan ..... B41J 2/335

Primary Examiner—Huan Tran

Attorney, Agent, or Firm—Sughrue, Mion, Zinn, Macpeak  
& Seas, PLLC

## [57] ABSTRACT

There is provided a thermal head having protective layers comprising a lower protective layer, an intermediate layer and a carbon-based protective layer which is composed of a plurality of sub-layers, wherein the carbon-based protective layer has stress values that become sequentially higher from one of the sub-layers located undermost toward another of the sub-layers located uppermost. The protective layers have significantly reduced corrosion and wear and is protected from cracking and peeling, whereupon the thermal head obtained can have sufficient durability and reliability to ensure that thermal recording of high-quality images is consistently performed over an extended period of operation.

2 Claims, 1 Drawing Sheet



FIG. 1



FIG. 2



## THERMAL HEAD

## BACKGROUND OF THE INVENTION

This invention relates to the art of thermal heads for thermal recording which are used in various types of printers, plotters, facsimile, recorders and the like as a recording device.

Thermal materials comprising a thermal recording layer on a substrate of a film or the like are used to record images produced in diagnosis by ultrasonic scanning (sonography).

This recording method, also referred to as thermal recording, eliminates the need for wet processing and offers several advantages including convenience in handling. Hence in recent years, the use of the thermal recording system is not limited to small-scale applications such as diagnosis by ultrasonic scanning and an extension to those areas of medical diagnoses such as CT, MRI and X-ray photography where large and high-quality images are required is under review.

As is well known, thermal recording involves the use of a thermal head having a glaze, in which heating elements comprising heaters and electrodes, used for heating a thermal material to record an image are arranged in one direction (main scanning direction) and, with the glaze urged at small pressure against the thermal material, the two members are moved relative to each other in the auxiliary scanning direction perpendicular to the main scanning direction, and energy is applied to the heating elements of the respective pixels in the glaze in accordance with image data to be recorded which were supplied from an image data supply source such as MRI or CT in order to heat the thermal recording layer of the thermal material, thereby performing image recording through color formation.

A protective film is formed on the surface of the glaze of the thermal head in order to protect the heaters for heating a thermal material, the associated electrodes and the like. Therefore, it is this protective film that contacts the thermal material during thermal recording and the heaters heat the thermal material through this protective film so as to perform thermal recording.

The protective film is usually made of wear-resistant ceramics; however, during thermal recording, the surface of the protective film is heated and kept in sliding contact with the thermal material, so it will gradually wear and deteriorate upon repeated recording.

If the wear of the protective film progresses, density unevenness will occur on the thermal image or a desired protective strength can not be maintained and, hence, the ability of the protective film to protect the heaters is impaired to such an extent that the intended image recording is no longer possible (the head has lost its function).

Particularly in the applications such as the aforementioned medical use which require multiple gradation images of high quality, the trend is toward ensuring the desired high image quality by adopting thermal films with highly rigid substrates such as polyester films and also increasing the setting values of recording temperature (energy applied) and of the pressure at which the thermal head is urged against the thermal material. Under these circumstances, as compared with the conventional thermal recording, a greater force and more heat are exerted on the protective film of the thermal head, making wear and corrosion (or wear due to corrosion) more likely to progress.

With a view to preventing the wear of the protective film on the thermal head and improving its durability, a number

of techniques to improve the performance of the protective film have been considered. Among others, a carbon-based protective film (hereinafter referred to as a carbon protective layer) is known as a protective film excellent in resistance to wear and corrosion.

Thus, Examined Published Japanese Patent Applications (KOKOKU) No. 61-53955 and No. 4-62866 (the latter being the divisional application of the former) disclose a thermal head excellent in wear resistance and response which is obtained by forming a very thin carbon protective layer having a Vickers hardness of 4500 kg/mm<sup>2</sup> or more as the protective film of the thermal head and a method of manufacturing the thermal head, respectively.

Unexamined Published Japanese Patent Application (KOKAI) No. 7-132628 discloses a thermal head which has a dual protective film comprising a lower silicon-based compound layer and an overlying diamond-like carbon layer, said protective film having wear and breakage significantly reduced, thereby ensuring that high-quality images can be recorded over an extended period of time.

The carbon protective layer has properties quite similar to those of diamond including a very high hardness and chemical stability, hence the carbon protective layer presents sufficiently excellent properties to prevent wear and corrosion which may be caused by the sliding contact with thermal materials.

The carbon protective layer is excellent in wear resistance, but brittle because of its hardness, that is, low in tenacity. Therefore, a thermal shock or stress due to heating of heating elements, a stress due to a difference in the coefficient of thermal expansion between the carbon protective layer and the neighboring layer, a mechanical impact due to a foreign matter entered between the thermal material and the thermal head (glaze) during recording, or other factors may bring about rather easily cracking or peeling.

If cracking or peeling is caused in the protective layer, wear, corrosion and also wear due to corrosion progress, leading to the reduction of the durability of the thermal head. The thermal head is not capable of exhibiting high reliability over an extended period of time.

## SUMMARY OF THE INVENTION

An object of the present invention is to solve the above problems in the prior art by providing a thermal head having a carbon-based protective layer, said protective layer having significantly reduced corrosion and wear and being protected from cracking and peeling due to heat or a mechanical impact, thereby enabling the thermal head to have a sufficient durability to ensure that high reliability can be exhibited over an extended period of time to perform thermal recording of high-quality images consistently over an extended period of operation.

In order to achieve the above object, the invention provides a thermal head having protective layers of heating elements, said protective layers comprising a lower protective layer, an intermediate protective layer formed on said lower protective layer, and a carbon-based protective layer which is composed of a plurality of sub-layers and formed on said intermediate protective layer, wherein said carbon-based protective layer has stress values that become sequentially higher from one of said sub-layers located undermost toward another of said sub-layers located uppermost.

In a preferred embodiment, the lower protective layer is a ceramic protective layer, and the intermediate protective layer is based on at least one component selected from a group consisting of metals of Groups IVA, VA and VIA, and silicon and germanium.

## BRIEF DESCRIPTION OF THE DRAWINGS

FIG. 1 is a schematic cross sectional view showing the structure of a heating element in the thermal head of the invention; and

FIG. 2 shows the concept of an exemplary film deposition apparatus for use in fabricating the thermal head of the invention.

## DETAILED DESCRIPTION OF THE INVENTION

The thermal head of the invention will now be described in detail with reference to the preferred embodiments shown in the accompanying drawings.

FIG. 1 shows a schematic cross sectional view of a heating element in the thermal head of the invention.

The thermal head 10 shown in FIG. 1 is capable of image recording on thermal sheets of up to, for example, B4 size at a recording (pixel) density of, say, about 300 dpi. Except for the protective layers, the head has a known structure in that heating elements performing thermal recording on a thermal material A are arranged in one direction, that is, in a main scanning direction (which is normal to the plane in FIG. 1).

It should be noted that the thermal head 10 of the invention is not particularly limited in such aspects as the width (in the main scanning direction), resolution (recording density) and recording gradation; preferably, the head width ranges from 5 cm to 50 cm, the resolution is at least 6 dots/mm (ca. 150 dpi), and the recording gradation consists of at least 256 levels.

The thermal material A used for thermal recording in the thermal head 10 of the invention is of an ordinary type which comprises a substrate of a transparent polyethylene terephthalate (PET) film or the like which is overlaid with a thermal recording layer. A material containing a lubricant is preferably used as the thermal material A in such an aspect as preferred sticking reduction.

As shown in FIG. 1, to form the thermal head 10, the top of a substrate 12 (which is shown to face down in FIG. 1 since the thermal head 10 is pressed downward against the thermal material A) is overlaid with a glaze layer (heat accumulating layer) 14 which, in turn, is overlaid with a heater (heat-generating resistor) 16 which, in turn, is overlaid with electrodes 18 which, in turn, is overlaid with protective layers which protect the heating element comprising the heater 16 and the electrodes 18, and the like.

The protective layers in the illustrated thermal head 10 are composed of three layers: a lower protective layer 20 superposed on the heater 16 and the electrodes 18, an intermediate protective layer (hereinafter referred to as an intermediate layer) 22 formed on the lower protective layer 20 and a carbon-based protective layer (hereinafter referred to as a carbon protective layer) 28 which are formed on the intermediate layer 22 and which comprises a plurality of sub-layers, or a first carbon protective sub-layer 24 and a second carbon protective sub-layer 26.

The thermal head 10 of the invention has essentially the same structure as known versions of thermal head except for the protective layers. Therefore, the arrangement of other layers and the constituent materials of the respective layers are not limited in any particular way and various known versions may be employed. Specifically, the substrate 12 may be formed of various electrical insulating materials including heat-resistant glass and ceramics such as alumina, silica and magnesia; the glaze layer 14 may be formed of

heat-resistant glass, heat resistant resins including polyimide resin and the like; the heater 16 may be formed of heat-generating resistors such as Nichrome (Ni—Cr), tantalum metal and tantalum nitride; and the electrodes 18 may be formed of electrically conductive materials such as aluminum, gold, silver and copper.

Heating elements on the glaze are known to be available usually in two types, one being of a thin-film type which is formed by a "thin-film" process such as vacuum evaporation, chemical vapor deposition (CVD) or sputtering and a photoetching technique, and the other being of a thick-film type which is formed by a "thick-film" process comprising the steps of printing (e.g., screen printing) and firing. The thermal head 10 for use in the invention may be formed by either method.

The material of the lower protective layer 20 to be formed in the thermal head 10 of the invention is not limited in any particular way and the lower protective layer 20 may be formed of a variety of known materials as long as they have sufficient heat resistance, corrosion resistance and wear resistance to serve as the protective layer of the thermal head. A variety of ceramic materials are preferably used.

Specific materials include silicon nitride ( $Si_3N_4$ ), silicon carbide (SiC), tantalum oxide ( $Ta_2O_5$ ), aluminum oxide ( $Al_2O_3$ ), SIALON (Si—Al—O—N), LASION (La—Si—O—N), silicon oxide ( $SiO_2$ ), aluminum nitride (AlN), boron nitride(BN), selenium oxide (SeO), titanium nitride (TiN), titanium carbide (TiC), titanium carbide nitride (TiCN), chromium nitride (CrN) and mixtures thereof. Among others, nitrides and carbides are preferably used in such aspects as easy film deposition, manufacturing cost, and resistance to mechanical wear and chemical wear. Silicon nitride, silicon carbide and SIALON are more preferably used. Additives such as metals may be incorporated in small amounts into the lower protective layer 20 to adjust physical properties thereof.

Methods of forming the lower protective layer 20 are not limited in any particular way and known methods of forming ceramic layers may be employed by applying the aforementioned thick-film and thin-film processes and the like. Among those methods, CVD is preferably employed.

As is well known, CVD is a technique of film deposition in which thermal or optical energy is applied to gaseous materials in a reaction chamber to induce various chemical reactions, thereby depositing substances on the substrate. The lower protective layer 20 which is very fine and has no defects such as cracks can be formed by means of CVD, whereupon a thermal head more excellent in durability and advantageous in image quality can be obtained.

The thickness of the lower protective layer 20 is not limited to any particular value but it ranges preferably from about 0.2  $\mu m$  to about 20  $\mu m$ , more preferably from about 2  $\mu m$  to about 15  $\mu m$ . If the thickness of the lower protective layer 20 is within the stated ranges, preferred results are obtained in various aspects such as the balance between wear resistance and heat conductivity (that is, recording sensitivity).

The lower protective layer 20 may comprise multiple sub-layers. In this case, multiple sub-layers may be formed of different materials or multiple sub-layers different in density may be formed of one material. Alternatively, the two methods may be combined to obtain sub-layers.

The thermal head 10 shown in FIG. 1 has a three protective layers which comprise the lower protective layer 20 as described above, the intermediate layer 22 formed on the lower protective layer 20, and the carbon protective layer

**28** (first and second carbon protective sub-layers **24, 26**) formed on the intermediate layer **22**.

The carbon protective layer **28** has chemically high stability as described above. Hence, the carbon protective layer **28** provided on the lower protective layer **20** advantageously protects the lower protective layer **20**, the electrodes **18**, the heater **16** and the like from chemical corrosion, and prolongs the service life of the thermal head **10**. If the intermediate layer **22** is further formed therebetween, the adhesion of the carbon protective layer **28** to the lower protective layer **20** and the shock absorption thereof are improved, whereupon a thermal head having more prolonged service life and more excellent in durability and long-term reliability can be obtained.

The intermediate layer **22** formed on the thermal head **10** is preferably based on at least one component selected from the group consisting of metals in Group IVA (titanium group), Group VA (vanadium group) and Group VIA (chromium group) of the periodic table, as well as silicon (Si) and germanium (Ge) in such aspects as the adhesion between the upper carbon protective layer **28** and the lower protective layer **20** and the durability of the carbon protective layer **28**.

Preferred specific examples include Si, Ge, titanium (Ti), tantalum (Ta), molybdenum (Mo) and mixtures thereof. Among others, Si and Mo are more preferably used in the binding with carbon and other aspects. Most preferably, Si is used.

Methods of forming the intermediate layer **22** are not limited in any particular way and any known film deposition methods may be used in accordance with the material of the intermediate layer **22** by applying the aforementioned thick-film and thin-film processes and the like. A preferred method includes sputtering, but plasma-assisted CVD is also available with advantage.

The intermediate layer **22** may also comprise multiple sub-layers. In this case, multiple sub-layers may be formed of different materials or multiple sub-layers different in density may be formed of one material. Alternatively, the two methods may be combined to obtain sub-layers.

Prior to forming the intermediate layer **22**, lapping treatment, etching treatment and the like may be performed on the surface of the lower protective layer **20**. Thus, the adhesion between the lower protective layer **20** and the intermediate layer **22** and the adhesion between the intermediate layer **22** and the carbon protective sub-layer **24** in the carbon protective layer can be improved, leading to the improvement in the durability of the thermal head.

The surface roughness of the lower protective layer **20** in these treatments is not limited to any particular value, but the surface roughness expressed by "Ra" value is preferably in the range of from 1 nm to 0.1  $\mu$ m.

In the illustrated thermal head **10**, the intermediate layer **22** is overlaid with the first carbon protective sub-layer **24** containing carbon as a main component. Then, the sub-layer **24** is overlaid with the second carbon protective sub-layer **26** also containing carbon as a main component. The stress values of the two carbon protective sub-layers **24, 26** are different. The second carbon protective sub-layer **26** located above has a higher stress value than the first carbon protective sub-layer **24**.

As described above, the carbon protective layer **28** having chemically high stability effectively protects the lower protective layer **20** from chemical corrosion and advantageously improves the durability of the thermal head **10**. In the present invention having a structure in which the plu-

rality of carbon protective sub-layers **24, 26** being formed have stress values which become sequentially larger toward the top sub-layer **26**, the adhesion of the carbon protective layer **28** to the intermediate and lower protective layers **22, 20** located below are improved, and the carbon protective layer **28** is protected from cracking and peeling caused by a thermal shock or stress, a stress due to a difference in the coefficient of thermal expansion between the carbon protective layer and the lower layers and a mechanical impact due to a foreign matter as described above. Thus, a thermal head having more prolonged service life and more excellent in durability and reliability is obtained.

It should be noted that the carbon-based protective layer as used in the present invention refers to a carbon layer containing not less than 50 atm % of carbon, and preferably comprising carbon and inevitable impurities. In the thermal head of the invention, suitable components to be incorporated in addition to carbon to form the carbon protective layer include hydrogen, nitrogen, fluorine, Si and Ti. In the case of hydrogen, nitrogen and fluorine, the content thereof in the carbon protective layer is preferably less than 50 atm %, and in the case of Si and Ti, the content thereof in the carbon protective layer is preferably not more than 20 atm %.

In the thermal head **10** of the invention, the stress of the carbon protective layer is not limited to any particular value, but the stress of the carbon protective sub-layer **26** located uppermost is preferably about two times to about ten times that of the carbon protective sub-layer **24** located undermost.

The stress of a thin film can be calculated by the following equation:

$$S = dED^2/[3L^2(1-v)]$$

where "S" represents the stress of a thin film, "E" the Young's modulus of the substrate, "v" the Poisson's ratio of the substrate, "D" the thickness of the substrate, "L" the length of the thin film, and "d" the deflection amount of the substrate, respectively. Hence, the stress values of the carbon protective sub-layers can be compared by the deflection amount of the substrate having a deposited film for instance. The larger the deflection amount is, the higher the stress is.

Further, the number of the carbon protective sub-layers is not limited in any particular way, if the carbon protective layer comprises more than one carbon protective sub-layer. Two to five sub-layers are preferred in such aspects as the productivity of the thermal head and the adhesion between the respective sub-layers.

Methods of forming the carbon protective layer are not limited in any particular way and any known film deposition methods may be used in accordance with the composition of the carbon protective layer to be formed. Preferred methods include sputtering, especially magnetron sputtering, and CVD, especially plasma-assisted CVD.

When using the aforementioned film deposition devices, conditions for film deposition can be adjusted to form the plurality of carbon protective sub-layers **24, 26** having different stress values as described above.

When forming the carbon protective sub-layers **24, 26** by sputtering for example, the degree of vacuum (internal pressure of the system) during film deposition can be adjusted to adjust the hardness of the carbon protective sub-layers **24, 26**. Specifically, a carbon protective sub-layer having a higher hardness or a higher stress can be formed by increasing the degree of vacuum.

The stress of the carbon protective sub-layers **24, 26** can also be adjusted by adjusting the flow rate of hydrogen gas

being introduced together with a plasma generating gas. Specifically, in case of using argon as the plasma generating gas, film deposition of the carbon protective sub-layer having the highest hardness is achieved when the flow rate of the hydrogen gas is 5 to 10% of that of the argon. The layer becomes softer with the increase of the hydrogen amount. Then, this relationship can be utilized to form the plurality of carbon protective sub-layers 24, 26 having different stress values.

Methods of controlling the stress of the carbon protective sub-layers 24, 26 in sputtering film deposition are not limited in any particular way, and the carbon protective sub-layers 24, 26 having desired stress values can be formed for example in accordance with the relationship between the degree of vacuum during film deposition or the flow rate of the hydrogen gas and the hardness of the layer which was previously determined by an experiment or the like.

When forming the carbon protective sub-layers 24, 26 by CVD, the bias voltage to be applied to the thermal head having the substrate can be adjusted to form the carbon protective sub-layers 24, 26 having different stress values.

As is well known, film deposition by CVD is preferably performed with a negative bias voltage being applied to the substrate. In general, in the carbon protective sub-layers 24, 26 being deposited by CVD while applying a negative bias voltage to the substrate, the hardness is raised with the increase of the negative bias voltage from zero to reach the highest value at the bias voltage in the range of from -200V to -300V. However, when the negative bias voltage exceeds the above range, the hardness begins to decrease to the contrary. Therefore, this relationship can be utilized to form the plurality of carbon protective sub-layers 24, 26 having different stress values.

Methods of controlling the stress of the carbon protective sub-layers 24, 26 in CVD film deposition are not limited in any particular way, and the carbon protective sub-layers 24, 26 having desired stress values can be formed as in sputtering described above, for example in accordance with the relationship between the bias voltage during film deposition and the hardness of the layer which was previously determined by an experiment or the like.

The carbon protective layer 28 (sub-layers 24, 26) may be formed while heating to about 50°C.-400°C., especially to a temperature at which the thermal head 10 is used. In this method, the adhesion of the carbon protective layer to the intermediate layer 22 and the lower protective layer 20 can be further improved, and more excellent durability can be imparted to the carbon protective layer 28 which is protected from cracking and peeling caused by a thermal shock and a mechanical impact due to a foreign matter entered during thermal recording, as well as alteration and attrition due to high power recording. It should be however noted that heating can be performed by a method using a heating device such as a heater, or a method of energizing the thermal head.

The hardness of the carbon protective layer 28 is not limited to any particular value as far as the carbon protective layer has a sufficient hardness to serve as the protective layer of the thermal head. Thus, in the illustrated carbon protective layer 28 comprising two carbon sub-layers, the first carbon protective sub-layer 24 on the lower side has advantageously a Vickers hardness of about from 1000 kg/mm<sup>2</sup> to 2000 kg/mm<sup>2</sup>, and the second carbon protective sub-layer 26 on the upper side has advantageously a Vickers hardness of about from 2000 kg/mm<sup>2</sup> to 3000 kg/mm<sup>2</sup>.

In the thermal head 10 of the invention comprising the lower protective layer 20, the intermediate layer 22 and the

carbon protective layer 28 including the plurality of sub-layers 24, 26, the intermediate layer 22 and the carbon protective layer 28 are not limited in thickness to any particular values. The intermediate layer 22 has preferably a thickness of from 0.05 μm to 1 μm, more preferably from 0.1 μm to 1 μm. The carbon protective layer has preferably a total thickness of from 0.5 μm to 5 μm, especially from 1 μm to 3 μm. In the illustrated carbon protective layer 28 having two carbon sub-layers, both of the first carbon protective sub-layer 24 located below and the second carbon protective sub-layer 26 located above have preferably a thickness of 0.5 μm to 1.5 μm.

In the case of the intermediate layer 22 which is much thicker than the carbon protective layer 28, cracking and peeling may often take place in the intermediate layer 22. When the intermediate layer 22 is much thinner than the carbon protective layer 28, the intermediate layer 22 can not exhibit sufficient functions to be performed as the intermediate layer 22. Therefore, if the thickness values of the intermediate layer 22 and the carbon protective layer are within the stated ranges, the adhesion of the intermediate layer 22 to the lower protective layer 20 and the shock absorption thereof as well as the functions of the carbon protective layer 28 including durability can be consistently realized in a well balanced manner.

It should be however noted that the protective layers formed on the thermal head of the invention are not limited to the structure as described above, and a variety of structures can be used, as far as the protective layers have the lower protective layer 20, the intermediate layer 22 and the carbon protective layer 28 comprising the plurality of carbon protective sub-layers 24, 26, and the stress values of the sub-layers 24, 26 become sequentially larger from the bottom sub-layer 24 toward the top sub-layer 26 of the carbon protective layer 28.

Thus, after the carbon protective layer 28 is formed, a lubricant or wax may be applied to the surface thereof, and where appropriate, be baked by heating with a heater or by driving the thermal head. In this case, application and baking of the lubricant or wax can be performed after the carbon protective layer 28 is etched with oxygen. The lubricant and the wax are not limited in any particular way, and a variety of types can be used. For example, a lubricant contained in the thermal material A, a coating agent having heat resistance, preferably a coating agent excellent in lubricating properties are available.

FIG. 2 shows the concept of a film deposition apparatus suitable for forming the protective layers of the thermal head of the invention.

The illustrated film deposition apparatus generally indicated by 50 in FIG. 2 comprises a vacuum chamber 52, a gas introducing section 54, a first sputter device 56, a second sputter device 58, a plasma generating device 60, a bias source 62 and a substrate holder 64 as the basic components.

The film deposition apparatus 50 comprises three film deposition devices located in the system or the vacuum chamber 52, the two being performed by sputtering and the other by plasma-assisted CVD. A plurality of layers which are different in the composition can be formed continuously without opening the system.

Therefore, the film deposition apparatus 50 can be used to form easily the intermediate layer 22 (or the lower protective layer 20) and the carbon protective layer 28 with a high efficiency by means of sputtering using different targets or the combination of sputtering with plasma-assisted CVD.

The vacuum chamber 52 is preferably formed of a non-magnetic material such as SUS 304. A vacuum pump-down

device 66 is provided to evacuate the interior of the film deposition system to depress the pressure. Those sites of the vacuum chamber 52 where plasma develops or an arc is produced by plasma generating electromagnetic waves may be covered with an insulating member, which may be made of insulating materials including MC nylon, Teflon (PTFE) or the like.

The gas introducing section 54 consists of two parts 54a and 54b, the former being a site for introducing a plasma generating gas and the latter for introducing a reactive gas for use in the plasma-assisted CVD, into the vacuum chamber 52.

Inert gases such as helium, neon and the like are used as the plasma generating gas. Examples of the reactive gas for producing the carbon protective layer are the gases of hydrocarbon compounds such as methane, ethane, propane, ethylene, acetylene and benzene. Examples of the reactive gas for producing the intermediate layer 22 are various gases including materials used to form the intermediate layer 22.

To effect sputtering, a target 70 to be sputtered is placed on each of cathodes 68 and 76, which are rendered at negative potential and a plasma is generated on the surface of the target 70, whereby atoms are struck out of the target 70 and deposit on the surface on the opposed substrate to form the layer.

The first sputter device 56 and the second sputter device 58 are intended for sputtering film deposition on the surface of the substrate. The former comprises the cathode 68, the area where the target 70 is to be placed, a shutter 72, a radio-frequency (RF) power supply 74 and other components. The latter comprises the cathode 76, the area where the target 70 is to be placed, a shutter 78, a direct current (DC) power supply 80 and other components.

As seen from the above configuration, the first sputter device 56 and the second sputter device 58 have basically a similar configuration except that the power supply and the positions of the respective components are different. Therefore, we now describe the first sputter device 56 as a typical example except for the different portions.

The output and performance of the two power supplies are not limited in any particular way, and a device having the necessary and sufficient performance to produce a desired layer can be selected. Thus, in the case of an apparatus used to form the intermediate layer 22 and the carbon protective layer as described above, an RF power supply having a frequency of 13.56 MHz and producing a maximal output of 5 kW, and a DC power supply which is at negative potential capable of producing a maximal output of 10 kW can be used as the RF power supply 74 and the DC power supply 80, respectively. At least one of the two power supplies, especially the one used to form the carbon protective layer is preferably combined with a modulator to enable pulse modulation at frequencies in the range of 2 to 100 kHz. Thus, voltage inversion can be performed when an arc discharge is detected during formation of the carbon protective layer 28 or the like, whereupon the carbon protective layer 28 or the like can be formed more advantageously.

In the illustrated case, a backing plate 82 (or 84 in the second sputter device 58) made of oxygen-free copper, stainless steel or the like is first fixed to the cathode 68 and the target 70 is then attached to the backing plate 82 with In-based solder or by a mechanical fixing device. Preferred materials of the target 70 used to form the intermediate layer 22 include metals of the Groups IVA, VA and VIA and monocrystalline Ge and Si and the like. The target 70 used to form the carbon protective layer is preferably made of sintered carbon, glassy carbon or the like.

The illustrated apparatus 50 performs magnetron sputtering, in which magnets 68a (or 76a) are placed within the cathode 68 and a sputtering plasma is confined within a magnetic field formed on the surface of the target 70. Magnetron sputtering is preferred since it achieves high deposition rates.

The illustrated film deposition apparatus 50 is used to form the carbon protective layer 28 or the like by means of the plasma-assisted CVD with microwave ECR discharge which generate plasma with microwave in the ECR magnetic field. The plasma generating device 60 comprises a microwave source 86, magnets 88, a microwave guide 90, a coaxial transformer 92, a dielectric plate 94 and a radial antenna 96 and the like.

A source having the necessary and sufficient output to produce the carbon protective layer 28 and the like can appropriately be selected as the microwave source 86. Permanent magnets or electromagnets capable of forming a desired magnetic field can be appropriately used as the magnets 88 for generating the ECR magnetic field. The microwave is introduced into the vacuum chamber 52 by means of the microwave guide 90, the coaxial transformer 92, the dielectric plate 94 and the like.

The substrate holder 64 is used to fix the portion to be coated with the protective layers in the thermal head 10 (or the substrate) in position. The film deposition apparatus 50 as shown in FIG. 2 comprises these three film deposition devices. The substrate holder 64 is held on a rotary base 98 which rotates to move the substrate holder 64 so that the glaze on the substrate holder 64 can be opposed to the respective film deposition devices, that is, the sputter devices 56 and 58, and the plasma generating device 60 performing the plasma-assisted CVD.

The distance between the substrate holder 64 and the target 70 or the radial antenna 96 can be adjusted by a known method and a distance that provides a uniform thickness profile may be set appropriately.

As described above, the surface of the lower protective layer 20 or the intermediate layer 22 is roughened as required by etching. In addition, film deposition is preferably performed with a negative bias voltage being applied to the substrate in order to obtain a hard layer by the plasma-assisted CVD.

To do this, the bias source 62 that applies a radio-frequency voltage to the substrate is connected to the substrate holder 64 in the film deposition apparatus 50. A radio-frequency self-bias voltage is preferably used in the plasma-assisted CVD.

On the foregoing pages, the thermal head of the invention has been described in detail but the present invention is in no way limited to the stated embodiments and various improvements and modifications can of course be made without departing from the spirit and scope of the invention.

As described above in detail, the present invention provides a thermal head with prolonged service life, said thermal head having protective layers which have significantly reduced corrosion and wear and which allow the thermal head to have sufficient durability and reliability to ensure that thermal recording of high-quality images is consistently performed over an extended period of operation.

The invention will be further illustrated by means of the following specific example.

#### EXAMPLE 1

As in known methods of fabricating a thermal head, the substrate 12 was overlaid with the heat accumulating layer

14 which, in turn, was overlaid with the heater 16 which, in turn, was overlaid with the electrodes 18. Then, a silicon nitride ( $\text{Si}_3\text{N}_4$ ) layer having a thickness of 4  $\mu\text{m}$  was formed thereon by a conventional sputtering. Thus, the thermal head used as the base was fabricated.

Therefore, in Example 1, the silicon nitride layer corresponds to the lower protective layer 20, which is overlaid with the intermediate layer 22 which, in turn, is overlaid with the carbon protective layer 28.

The film deposition apparatus 50 shown in FIG. 2 and described below was used to form the intermediate layer 22, and the first and second carbon protective sub-layers 24, 26 on the thermal head as described above.

The film deposition apparatus 50 is now described in detail.

a. Vacuum Chamber 52

The vacuum chamber 52 made of SUS 304 and having a capacity of 0.5  $\text{m}^3$  was used; the vacuum pump-down device 66 comprised one unit each of a rotary pump having a pumping speed of 1,500 L/min, a mechanical booster pump having a pumping speed of 12,000 L/min and a turbomolecular pump having a pumping speed of 3,000 L/sec. An orifice valve was fitted at the suction inlet of the turbomolecular pump to allow for 10 to 100% adjustment of the degree of opening.

b. Gas Introducing Section 54

A mass flow controller permitting a maximum flow rate of 100 to 500 sccm and a stainless steel pipe having a diameter of 6 mm were used to form two gas introducing parts 54a and 54b, the former being used for introducing a plasma generating gas and the latter being used for introducing a reactive gas.

c. First and Second Sputter Devices 56, 58

The cathodes 68 and 76 used were in a rectangular form having a width of 600 mm and a height of 200 mm, with Sm—Co magnets being incorporated as the permanent magnets 68a and 76a.

The backing plates 82 and 84 were rectangular oxygen-free copper members, which were attached to the cathodes 68 and 76 with In-based solder. The interior of the cathodes 68 and 76 was water-cooled to cool the magnets 68a and 76a, the cathodes 68 and 76 and the rear side of each of the backing plates 82 and 84.

The RF power supply 74 used had a frequency of 13.56 MHz and could produce a maximal output of 5 kW. The DC power supply 80 used was at negative potential capable of producing a maximal output of 10 kW. The DC power supply 80 was adapted to be capable of pulse modulation at frequencies in the range of 2 to 100 kHz in combination with the modulator.

d. Plasma Generating Device 60

The microwave source 86 oscillating at a frequency of 2.45 GHz and producing a maximal output of 1.5 kW was employed. The generated microwave was guided to the neighborhood of the vacuum chamber 52 by means of the microwave guide 90, converted in the coaxial transformer 92 and directed to the radial antenna 96 in the vacuum chamber 52.

The plasma generating part used was in a rectangular form having a width of 600 mm and a height of 200 mm.

In addition, a magnetic field for ECR was produced by arranging a plurality of Sm—Co magnets used as the magnets 88 in a pattern to conform to the shape of the dielectric plate 94.

e. Substrate Holder 64

The rotary base 98 was rotated to move the substrate holder 64 so that the substrate (the thermal head 10) fixed

thereon is kept opposed to one of the targets 70 in the first and second sputter devices 56 and 58 and the radial antenna 96 in the plasma generating device 60.

The distance between the substrate and each target 70 was set at 100 mm when forming the intermediate layer 22 and the carbon protective layer by sputtering as described below.

In addition, the area of the substrate holder 64 in which the thermal head was held was set at a floating potential in order to enable the application of an etching radio-frequency voltage. A heater was also provided on the surface of the substrate holder 64 for film deposition with heating.

f. Bias Source 62

An RF power supply was connected to the substrate holder 64 via the matching box.

15 The RF power supply had a frequency of 13.56 MHz and could produce a maximal output of 3 kW. It was also adapted to be such that by monitoring the self-bias voltage, the RF output could be adjusted over the range of -100 to -500 V.

In this apparatus 50, the bias source 62 also serves as the etching means.

Formation of Thermal Head 10:

In the film deposition apparatus 50 described above, the thermal head 10 used as the base was secured to the substrate holder 64 such that the heating elements would be kept 20 opposed to the target 70 positioned in the first sputter device 56. All areas of the thermal head other than those where the intermediate layer 22 was to be formed were previously 25 masked.

With continued pump-down, argon gas was introduced 30 through the gas introducing section 54 and the pressure in the vacuum chamber 52 was adjusted to 5.0 mTorr by means of the orifice valve fitted on the turbomolecular pump. Subsequently, a radio-frequency voltage was applied to the substrate and the lower protective layer 20 (silicon nitride layer) was etched for 10 minutes at a self-bias voltage of 35 -300 V.

After the end of etching, a monocrystalline silicon target and a sintered graphite member were fixed (i.e., attached by means of In-based solder) on the backing plate 82 in the first 40 sputter device 56 and on the backing plate 84 in the second sputter device 58, respectively. Then, the vacuum chamber 52 was evacuated again until the internal pressure reached  $5.0 \times 10^{-6}$  Torr. The argon gas flow rate and the orifice valve were adjusted so as to maintain the internal pressure in the 45 vacuum chamber 52 at 2.5 mTorr, and an RF power of 0.5 kW was applied to the target 70 for five minutes, with the shutter 72 being closed.

Subsequently, with the internal pressure in the vacuum chamber 52 kept at the stated level, the RF power was raised 50 to 2 kW and the shutter 72 was opened. The sputtering was performed to form a silicon layer having a thickness of 0.2  $\mu\text{m}$  as the intermediate layer 22.

To control the thickness of the silicon layer, the deposition rate was determined previously and the time required to 55 reach a specified layer thickness was calculated.

After the intermediate layer 22 was formed, the rotary base 98 was rotated to oppose the heating elements to the target 70 (i.e. the sintered graphite member) in the second sputter device 58. The argon gas flow rate and the orifice 60 valve were adjusted so as to maintain the internal pressure in the vacuum chamber 52 at 5 mTorr, and a DC power of 0.5 kW was applied to the target 70 for 5 minutes with the shutter 78 being closed.

Subsequently, with the internal pressure in the vacuum chamber 52 kept at the stated level, the DC power was raised 65 to 5 kW and the shutter 78 was opened. The sputtering was performed to form the first carbon protective sub-layer 24

having a thickness of 1  $\mu\text{m}$ . Then, the pressure in the vacuum chamber 52 was changed to 2.5 mTorr, and the sputtering was successively performed, with the supply power being kept unchanged. Thus, the second carbon protective sub-layer 26 having a thickness of 1  $\mu\text{m}$  was formed.

To control the thickness of the carbon protective sub-layers 24, 26 being formed, the deposition rate was determined previously and the time required to reach a specified layer thickness was calculated.

A carbon layer was previously formed on each of soft substrates, and the deflection amounts of the substrates were measured. A difference in the conditions for film deposition influencing the deflection amounts was found. Then, the stress of each carbon protective sub-layer was determined by reference to the difference. Specifically, a carbon layer having a thickness of 0.2  $\mu\text{m}$  was formed on the entire surface of each of polyethylene terephthalate (PET) films of 10 mmx50 mm having a thickness of 100  $\mu\text{m}$ , after which the deflection amounts of the PET films were measured. The conditions for film deposition were the same as in the above carbon protective layer except that three pressure values of 2.5 mTorr, 5.0 mTorr and 8.0 mTorr were applied to the vacuum chamber 52 to perform film deposition. Consequently, the deflection amounts of the PET films were in the range of about 3 to 30 mm, and increased in the order of 8.0 mTorr, 5.0 mTorr and 2.5 mTorr. That is, the deflection amount was inversely proportional to the pressure.

#### Evaluation of Performance:

The thus fabricated thermal head 10 was incorporated in the thermal recording apparatus, and thermal recording of a solid image was performed using a thermal material of B4 size (dry image recording film CRDP for medical application of Fuji Photo Film Co., Ltd.).

The result showed that the carbon protective sub-layers had no wear or delamination after image recording was performed on 40,000 sheets.

#### COMPARATIVE EXAMPLE 1

Example 1 was repeated except that a constant pressure of 2.5 mTorr was applied to the vacuum chamber 52 to form the carbon protective layer which comprised only one sub-layer having a thickness of 2  $\mu\text{m}$ . Thus, a thermal head having three protective layers was fabricated.

The thus obtained thermal head was used to perform the same thermal recording as in Example 1.

Consequently, image quality changed after recording was performed on 30,000 sheets or more, and delamination was confirmed in a portion of the carbon protective layer.

These results clearly demonstrate the effectiveness of the thermal head of the present invention.

What is claimed is:

1. A thermal head having protective layers of heating elements, said protective layers comprising a lower protective layer, an intermediate layer formed on said lower protective layer, and a carbon-based protective layer which is composed of a plurality of sub-layers and formed on said intermediate layer, wherein said carbon-based protective layer has stress values that become sequentially higher from one of said sub-layers located undermost toward another of said sub-layers located uppermost.

2. The thermal head according to claim 1, wherein said lower protective layer is a ceramic protective layer, and wherein said intermediate layer is based on at least one component selected from a group consisting of metals of Groups IVA, VA and VIA, and silicon and germanium.

\* \* \* \* \*

UNITED STATES PATENT AND TRADEMARK OFFICE  
**CERTIFICATE OF CORRECTION**

PATENT NO. : 6,061,077

DATED : May 09, 2000

INVENTOR(S) : Makoto KASHIWAYA, Junji NAKADA

It is certified that error appears in the above-identified patent and that said Letters Patent is hereby corrected as shown below:

**On the Title Page**

**SECOND INVENTOR:**

Please change the second inventor's last name: Junji [NAKATA] NAKADA

Signed and Sealed this

Seventeenth Day of April, 2001

Attest:



NICHOLAS P. GODICI

*Attesting Officer*

*Acting Director of the United States Patent and Trademark Office*